# EUROPEAN PATENT SPECIFICATION

(11) **EP 0 372 948 B1**
(45) Date of publication and mention of the grant of the patent: **29.06.1994**
(21) Application number: 89312748.0
(22) Date of filing: 07.12.1989
(51) Int. Cl.: H01F 1/053

(54) **Permanent magnet composition**
Dauermagnet-Zusammenstellung
Composition pour aimant permanent

(30) Priority: 08.12.1988 JP 308720/88
(43) Date of publication of application: 13.06.1990
(73) Proprietor: FUJI ELECTROCHEMICAL CO.LTD., Minatoku Tokyo 105 (JP)
(72) Inventor: Yasumura, Takaaki, Kosai-shi Shizuoka (JP); Kiyomiya, Teruo, Kosao-shi Shizuoka (JP); Mizuno, Yasutoshi, Toyohashi-shi Aichi (JP); Matsui, Kazuo, Toyohashi-shi Aichi (JP)
(74) Representative: Lewin, John Harvey

(56) References cited:
- US-A- 4 497 672
- CHEMICAL ABSTRACTS, vol. 93, no. 11, December 1980 Columbus, Ohio, USA S.Seikosha Co.: "Permanent magnet material" page 681; column 1; ref. no. 214498N
- PATENT ABSTRACTS OF JAPAN vol. 8, no. 25 (E-225)(1462) 2 February 1984,& JP-A-58 186906 (TOKYO SHIBAURA DENKI K.K.) 1 November 1983,
- PATENT ABSTRACTS OF JAPAN vol. 5, no. 103 (E-64)(775) 3 July 1981,& JP-A-56 46508 (SUWA SEIKOSHA K.K.) 27 April 1981,

## Description

### BACKGROUND OF THE INVENTION

### 1. Field of the Invention

The present invention relates to R₂M₁₇ (where R represents at least one of rare earth elements including yttrium and M is mainly transition metals) type permanent magnet composition and, more particularly, to the R₂M₁₇ type permanent magnet composition whose energy product is improved by increasing its residual magnetic flux density while maintaining its coercive force at a level equal to that obtainable in the prior art.

### 2. Description of Prior Art

In conventional R₂M₁₇ type permanent magnets using samarium as the rare earth element R and cobalt as the transition metal M the copper content is relatively large, above 10 weight percent, to obtain high coercive force (iHc) and iron is added to suppress deterioration of residual magnetic flux density (Br) which is caused when the copper content becomes large. In this instance, the amount of iron added is held less than about 8 weight percent, because the iron, if added in large quantity, would lower the residual magnetic flux density (Br).

However, the energy product (BH) obtainable with such a permanent magnet composition is only 175.9 KJ/m³ (22.1 MG·Oe)or so at the largest.

To increase the energy product (BH), a variety of permanent magnet compositions have been proposed so far.

Of the proposed compositions, (1) a composition which contains 22 wt% R, 5 to 12 wt% copper, 0.2 to 5 wt% X (which is at least one of niobium, zirconium, vanadium, tantalum, chromium, hafnium), 0.2 to 8 wt% manganese and the balance being cobalt which is substituted by less than 35 wt% iron (Japanese Patent Publication No. 56-11378), (2) a composition which contains 22 to 28 wt% R, 2 to 10 wt% copper, 6 to 35 wt% T (which is at least one of iron, manganese and chromium), 0.5 to 6 wt% M (zirconium and/or hafnium) and the balance being cobalt (Japanese Patent Publication No. 62-61665), and (3) a composition which is represented by the formula R (Co_{l-u-v-w} CuᵤFeᵥM_{w})_{z} where 0 < u ≦ 2, 0.01 < v ≦ 0.6, 0.005 ≦ w ≦ 0.05, 6.5 ≦ z < 8.8, and M is at least one element selected from the group consisting of tantalum, zirconium, niobium, titanium and hafnium (Japanese Patent Publication No. 61-17881) are high in both coercive force and residual magnetic flux density, and consequently, provide a great energy product.

All these compositions reduce the copper content but instead call for the addition of such expensive and difficult-to-get elements as tantalum, niobium and hafnium --this inevitably leads to advanced cost of material and hence eventually raises the manufacturing costs of products. Moreover, these compositions are all intended to provide a greater energy product by increasing both of the coercive force and the residual magnetic flux density. However, depending on the elements used, the coercive force increases while decreasing the residual magnetic flux density and vice versa as referred to above. Accordingly, it is very difficult to determine the particular composition which can raise both of characteristics.

Chemical Abstracts, vol. 93, no. 11, Dec. 1980, 214498n, discloses an R₂M₁₇ magnet given by the general formula R[Coₗ₋ᵤ₋ᵥ(Cu+Mn)ᵤFeᵥ]_{z} which can also contain the additional elements Zr, Zn, Bi and Al.

### SUMMARY OF THE INVENTION

It is therefore an object of the present invention to provide R₂M₁₇ type permanent magnet composition which reduced a copper content but instead uses low-cost, easily available elements and which provides a greater energy product by increasing a residual magnetic flux density and which has a higher coercive force than that in the prior art composition.

To attain the above objective, a permanent magnet composition of the present invention comprises 22 to 28% R (Where R represents at least one of rare earth elements including yttrium), 5 to 16% iron, 0.2 to 6.5% copper, 0.1 to 6% manganese, 1.0 to 4.0 A (where A represents at least one of zinc and zirconium), and 0.1 to 2% B (where B represents at least one of aluminum, bismuth and thallium) by weight, with the balance being cobalt.

### DESCRIPTION OF THE PREFERRED EMBODIMENTS

According to the present invention, the amount of copper, which is requisite to the R₂M₁₇ type permanent magnet composition, as well as R, iron and cobalt, is held small, i.e. between 0.2 and 6.5 weight percent. Instead, manganese, at least one of zinc and zirconium of the group A materials and at least one of aluminum, bismuth and thallium of the group B materials are added.

The zinc in group A and the aluminum in group B are low-cost and easily available and involves no significant difficulty in handling as is well known. With the permanent magnet composition of the present invention which substitutes the zinc and aluminum for the aforementioned hafnium, niobium, tantalum etc which are expensive, difficult to obtain and must be handled carefully, the coercive force (iHc) is about the same as that in the prior art compositions but the residual magnetic flux density (Br) is enhanced, providing for increased energy product, as will be seen from examples described later.

Incidentally, even if the zinc is partially or wholly replaced with the zirconium and the aluminum is partially or wholly replaced with bismuth and/or thallium, the same result can be obtained as described later.

The amount of the group A element should be between 1.0 and 4.0 weight percent because when its amount is less than 1.0 weight percent the coercive force is low, whereas when the amount exceeds 4.0 weight percent the residual magnetic flux density appreciably decreases and the coercive force also decreases.

If the group B element is greater than 2 weight percent, the residual magnetic flux density is not improved and the coercive force becomes lower than in the past. On the other hand, if the element is less than 0.1 weight percent, no effect is produced. Therefore, the amount of group B element must be in the range of 0.1 and 2 weight percent.

The reason the amount of the R is selected in the range of between 22 and 28 weight percent is that, if its amount is greater than 28 weight percent, the residual magnetic flux density decreases and hence its improvement (which is the object of the invention) cannot be attained, whereas when the amount of the R is less than 22 weight percent, the coercive force does not reach the value obtainable in the prior art compositions.

The manganese is added in amounts between 0.1 and 6 weight percent because no effect is produced if the manganese is less than 0.1 weight percent, whereas if it is greater than 6 weight percent, the coercive force and the residual magnetic flux density both decrease.

The copper should be added in amounts between 0.2 and 6.5 weight percent. If the copper is greater than 6.5 weight percent, the residual magnetic flux density lowers. On the other hand, if the copper content is less than 0.2 weight percent, the coercive force does not reach about the same level as in the prior art.

The iron is present in amounts between 5 and 16 weight percent. When the iron content is greater than 16 weight percent, the coercive force lowers as compared with that in the prior art. Also, if it is less than 5 weight percent, the residual magnetic flux density decreases.

The above-mentioned composition in accordance with the present invention are melted and casted into an ingot, which is finely pulverized into a powder. The powder is compression-molded into a desired shape at a pressure of 0.5 to 5 tons/cm² in a magnetic field having a field intensity between 398 and 1273 KA/m (5 and 16 kOe), thereafter the molding being subjected to the following heat treatment.

That is, the molding is sintered at 1180 to 1250°C for 1 to 10 hours, solution-treated at 1100 to 1240°C for 0.5 to 10 hours, subjected to a first aging treatment at 400 to 800°C for 0.5 to 5 hours and a second aging treatment at 750 to 950°C for 0.5 to 5 hours, and then cooled down to 600°C or below at a rate of 0.1 to 4°C/min.

In this way, a permanent magnet is obtained which has a coercive force about the same as that in the prior art composition but provides a greater energy product.

### EXAMPLE 1

Alloys of 24.1 wt% samarium, 3.9 wt% copper, 2.3 wt% zinc, 12.9 wt% iron, 2 wt% manganese, aluminum in amounts given in Table 1 and the balance cobalt were melted in a high-frequency melting furnace and roughly ground by a jaw crusher, thereafter being finely pulverized by a jet mill. The finely pulverized powders were compression-molded under a pressure of 3 tons/cm² in a magnetic field of 15 KOe field intensity. Then the moldings were sintered at 1180 to 1250°C for 5 hours, solution-treated at 1100 to 1240°C for 5 hours, and subjected to a first aging treatment at 700°C for 2 hours and a second aging treatment at 900°C for 3 hours. Finally, the moldings were cooled down to 400°C at a rate of 0.5°C/min.

The characteristics of the permanent magnets thus obtained are given in Table 1.

**Table 1**

| | | | | | |
|---|---|---|---|---|---|
| Al(wt%) | 0.5 | 1.0 | 1.5 | 2.0 | 2.5 |
| iHc (KA/m) | 868.99 | 860.23 | 853.87 | 849.89 | 819.65 |
| Br(T) | 1.103 | 1.124 | 1.114 | 1.104 | 1.082 |
| BHmax (KJ/m³) | 231.6 | 240.3 | 225.2 | 212.5 | 191.8 |

### EXAMPLE 2

Permanent magnets were produced in exactly the same manner as in Example 1 except that bismuth was used in amounts given in Table 2 in place of the aluminum used in Example 1.

The characteristics of the permanent magnets were as shown in Table 2.

**Table 2**

| | | | | | |
|---|---|---|---|---|---|
| Bi(wt%) | 0.5 | 1.0 | 1.4 | 2.0 | 2.5 |
| iHc (KA/m) | 829.20 | 820.44 | 806.92 | 798.96 | 748.03 |
| Br(T) | 1.104 | 1.120 | 1.130 | 1.125 | 1.114 |
| BHmax (KJ/m³) | 224.4 | 231.6 | 240.3 | 214.9 | 210.9 |

### EXAMPLE 3

Permanent magnets were produced in exactly the same manner as in Example 1 except that thallium was used in amounts given in Table 3 in place of the aluminum used in Exmple 1.

The characteristics of the permanent magnets are shown in Table 3.

**Table 3**

| | | | | | |
|---|---|---|---|---|---|
| Tl(wt%) | 0.5 | 1.0 | 1.5 | 2.0 | 2.5 |
| iHc (KA/m) | 868.99 | 860.23 | 851.48 | 840.34 | 833.18 |
| Br(T) | 1.104 | 1.114 | 1.122 | 1.127 | 1.103 |
| BHmax (KJ/m³) | 217.2 | 223.6 | 232.4 | 242.7 | 212.5 |

As will be appreciated from Tables 1 through 3, in case of using the thallium, even if its content is 2.5 weight percent which exceeds of the upper limit of the B element, i.e. 2 weight percent, the residual magnetic flux density (Br) is improved and a great energy product can be obtained. However, the thallium is so expensive that its content as large as 2.5 weight percent significantly raises the manufacturing costs of permanent magnets; consequently, it is preferable, from the economical point of view, that the upper limit of the thallium content is 2 weight percent.

### EXAMPLE 4

Alloys of 24.1 wt% samarium, 12.9 wt% iron, 3.9 wt% copper, 2 wt% manganese, zinc in amounts given in Table 4, 1.0 wt% aluminum and the balance cobalt prepared and permanent magnets were produced from the alloys in exactly the same manner as in Example 1.

The characteristics of the permanent magnets were as shown in Table 4.

**Table 4**

| | | | | |
|---|---|---|---|---|
| Zn(wt%) | 0.5 | 1.0 | 2.0 | 3.0 |
| iHc(KA/m) | 509.30 | 708.24 | 811.69 | 825.22 |
| Br(T) | 1.141 | 1.135 | 1.126 | 1.119 |
| BHmax (KJ/m³) | 183.03 | 224.4 | 237.9 | 232.4 |
| Zn(wt%) | 4.0 | 5.0 | 6.0 | 7.0 |
| iHc(KA/m) | 724.16 | 572.96 | 493.38 | 326.27 |
| Br(T) | 1.107 | 1.091 | 1.074 | 1.037 |
| BHmax (KJ/m³) | 223.6 | 200.5 | 175.87 | 136.1 |

In cases where the zinc content is 0.5 and 6.0 weight percent, the maximum energy product (BHmax) somewhat decreases as shown in Table 4, but such values still are sufficient for practical applications. Since the zinc is low-cost, readily available in the market and easy to handle, its addition is preferable from the economical point of view and in terms of productivity.

### EXAMPLE 5

An alloy of 24.1 wt% samarium, 12.9 wt% iron, 3.9 wt% copper, 2.0 wt% manganese, 1.1 wt% zinc, 0.9 wt% zirconium, 0.5 wt% aluminum, 0.1 wt% bismuth, 0.1 wt% thallium and the balance cobalt was prepared and a permanent magnet was produced in exactly the same manner as in Example 1.

The coercive force (iHc), the residual magnetic flux density (Br) and the maximum energy product (BHmax) of this permanent magnet were 836.36 KA/m, 1.110 T and 234.0 KJ/m³, respectively.

### EXAMPLE 6

Permanent magnets were produced in exactly the same manner as in Example 5 except that the bismuth or thallium was not added.

The coercive force (iHc), the residual magnetic flux density (Br) and the maximum energy product (BHmax) of the permanent magnet with no bismuth were 834.77 KA/m, 1.109 T and 232.4 KJ/m³, respectively. Also, the coercive force (iHc), the residual magnetic flux density (Br) and the maximum energy product (BHmax) of the permanent magnet with no thallium were 837.2 KA/m, 1.107 T and 233.2 KJ/m³, respectively.

### EXAMPLE 7

Alloys of 24.1 wt% samarium, 12.9 wt% iron, 3.9 wt% copper, manganese in amounts given in Table 5, 2.3 wt% zinc, 1.0 wt% aluminum and the balance cobalt were prepared and a permanent magnets were produced in exactly the same manner as in Example 1.

The characteristics of these permanent magnets are given in Table 5.

**Table 5**

| | | | | |
|---|---|---|---|---|
| Mn(wt%) | 0.5 | 1.0 | 2.0 | 3.0 |
| iHc(KA/m) | 835.56 | 821.24 | 806.92 | 798.96 |
| Br(T) | 1.089 | 1.104 | 1.130 | 1.110 |
| BHmax (KJ/m³) | 223.6 | 232.4 | 240.3 | 236.3 |
| Mn(wt%) | 4.0 | 5.0 | 6.0 | 7.0 |
| iHc(KA/m) | 796.57 | 794.18 | 719.38 | 628.66 |
| Br(T) | 1.097 | 1.089 | 1.084 | 1.069 |
| BHmax (KJ/m³) | 231.6 | 226.0 | 218.8 | 196.6 |

As described above in detail, the present invention provides permanent magnet compositions having improved energy product by raising the residual magnetic flux density while maintining the coercive force substantially at a level equal to that in the prior art compositions through use of aluminum, zinc and other elements which are low-cost, readily available and easy to handle. Thus, the present invention can remarkably reduce the manufacturing costs of permanent magnets.

Although the present invention has been described with reference to its preferred enbodiments and examples, it will be apparent that many modifications and variations may be effected without departing from the scope of the invention as defined in the claims.

## Claims

1. A permanent magnet composition comprising 22 to 28 wt% R, which is at least one of rare earth elements including yttrium; 5 to 16 wt% iron; 0.2 to 6.5 wt% copper; 0.1 to 6 wt% manganese; 1.0 to 4.0 wt% A, which is at least one of zinc and zirconium; 0.1 to 2 wt% B, which is at least one element selected from the group of aluminium, bismuth and thallium; and the balance being cobalt.

2. A permanent magnet composition comprising: 22 to 28 wt% R, R being at least one of rare earth elements including yttrium; 5 to 16 wt% iron; 0.2 to 6.5 wt% copper; 0.1 to 6 wt% manganese; 1.0 to 4.0 wt% A, A being at least one element selected from the group of zinc and zirconium; 0.1 to 2.5 wt% thallium; and the balance being cobalt.

3. A method of manufacturing a permanent magnet comprising the steps of:
preparing an alloy ingot comprising 22 to 28 wt% R, which is at least one of rare earth elements including yttrium; 5 to 16 wt% iron; 0.2 to 6.5 wt% copper; 0.1 to 6 wt% manganese; 1.0 to 4.0 wt% A, which is at least one of zinc and zirconium; 0.1 to 2 wt% B, which is at least one element selected from the group of aluminium, bismuth and thallium; and the balance being cobalt;
grinding the alloy ingot into fine powders;
compression-molding the powders into a predetermined shape at a pressure of 0.5 to 5 tons/cm² in a magnetic field having a field intensity between 5 and 16 KOe;
sintering the molding at a temperature between 1180 and 1250°C for a period between 1 and 10 hours;
solution-treating the molding at a temperature between 1100 and 1240°C for a period between 0.5 and 10 hours;
subjecting the molding to a first aging treatment at a temperature between 400 and 800°C for a period between 0.5 and 4 hours and then to a second aging treatment at a temperature between 750 and 950°C for a period beween 0.5 to 5 hours; and
cooling down the molding to below 600°C at a rate of 0.1 to 4°C/min.

## Patentansprüche

1. Dauermagnetzusammensetzung umfassend 22 bis 28 Gew.-% R, welches mindestens eines der Seltenerdelemente einschließlich von Yttrium ist; 5 bis 16 Gew.-% Eisen; 0,2 bis 6,5 Gew.-% Kupfer; 0,1 bis 6 Gew.-% Mangan; 1,0 bis 4,0 Gew.-% A, welches mindestens eines von Zink und Zirconium ist; 0,1 bis 2 Gew.-% B, welches mindestens ein Element, ausgewählt aus der Gruppe aus Aluminium, Bismut und Thallium ist; und wobei der Rest Kobalt ist.

2. Dauermagnetzusammensetzung umfassend 22 bis 28 Gew.-% R, wobei R mindestens eines der Seltenerdelemente einschließlich von Yttrium ist; 5 bis 16 Gew.-% Eisen; 0,2 bis 6,5 Gew.-% Kupfer; 0,1 bis 6 Gew.-% Mangan; 1,0 bis 4,0 Gew.-% A, wobei A mindestens ein Element, ausgewählt aus der Gruppe aus Zink und Zirconium ist; 0,1 bis 2,5 Gew.-% Thallium; und wobei der Rest Kobalt ist.

3. Verfahren zum Herstellen eines Dauermagneten umfassend die Schritte:
Herstellung eines Legierungsbarrens, umfassend 22 bis 28 Gew.-% R, welches mindestens eines der Seltenerdelemente einschließlich von Yttrium ist; 5 bis 16 Gew.-% Eisen; 0,2 bis 6,5 Gew.-% Kupfer; 0,1 bis 6 Gew.-% Mangan; 1,0 bis 4,0 Gew.-% A, welches mindestens eines von Zink und Zirconium ist; 0,1 bis 2 Gew.-% B, welches mindestens ein Element, ausgewählt aus der Gruppe aus Aluminium, Bismut und Thallium ist; und wobei der Rest Kobalt ist;
Mahlen des Legierungsbarrens zu feinen Pulvern;
Formpressen der Pulver zu einer vorbestimmten Gestalt bei einem Druck von 0,5 bis 5 t/cm² in einem Magnetfeld mit einer Feldstärke zwischen 5 und 16 KOe;
Sintern des Formkörpers bei einer Temperatur zwischen 1180 und 1250°C während eines Zeitraums zwischen 1 und 10 Stunden;
Lösungsbehandeln des Formkörpers bei einer Temperatur zwischen 1100 und 1240°C während eines Zeitraums zwischen 0,5 und 10 Stunden;
Unterwerfen des Formkörpers einer ersten Alterungsbehandlung bei einer Temperatur zwischen 400 und 800°C während eines Zeitraums zwischen 0,5 und 4 Stunden und dann einer zweiten Alterungsbehandlung bei einer Temperatur zwischen 750 und 950°C während eines Zeitraums zwischen 0,5 bis 5 Stunden; und
Abkühlen des Formkörpers auf unter 600°C mit einer Geschwindigkeit von 0,1 bis 4°C/min.

## Revendications

1. Une composition d'aimant permanent comprenant 22 à 28% en poids de R, qui est au moins un des éléments de terres rares incluant l'yttrium; 5 à 16% en poids de fer; 0,2 à 6,5% en poids de cuivre; 0,1 à 6% en poids de manganèse; 1,0 à 4,0% en poids de A, qui est au moins un parmi le zinc et le zirconium; 0,1 à 2% en poids de B qui est an moins un élément sélectionné dans le groupe de l'aluminium, du bismuth et du thallium; et l'équilibre étant le cobalt.

2. Une composition d'aimant permanent comprenant: 22 à 28% en poids de R, R étant au moins un des éléments de terres rares incluant l'yttrium; 5 à 16% en poids de fer; 0,2 à 6,5% en poids de cuivre; 0,1 à 6% en poids de manganèse; 1,0 à 4,0% en poids de A, A étant au moins un élément sélectionné dans le groupe du zinc et du zirconium; 0,1 à 2,5% en poids de thallium; et l'équilibre étant le cobalt.

3. Un procédé de fabrication d'un aimant permanent comprenant les étapes de:
préparation d'un lingot d'alliage comprenant 22 à 28% en poids de R, qui est au moins un des éléments de terres rares incluant l'yttrium; 5 à 16% en poids de fer; 0,2 à 6,5% en poids de cuivre; 0,1 à 6% en poids de manganèse; 1,0 à 4,0% en poids de A, qui est au moins un parmi le zinc et le zirconium; 0,1 à 2% en poids de B, qui est au moins un élément sélectionné dans le groupe de l'aluminium, du bismuth et du thallium; et l'équilibre étant le cobalt;
de broyage du lingot d'alliage en fine poudres;
de moulage par compression des poudres sous une forme prédéterminée à une pression de 0,5 à 5 tonnes/cm² dans un champs magnétique ayant une intensité de champs entre 5 et 16 kOe;
de frittage du moulage à une température entre 1180 et 1250°C pendant une période comprise entre 1 et 10 heures;
de recuisson par mise en solution du moulage à une température comprise entre 1100 et 1240°C pendant une période comprise entre 0,5 et 10 heures;
de soumission du moulage à un premier traitement de vieillissement à une température comprise entre 400 et 800°C pendant une période comprise entre 0,5 et 4 heures et ensuite à un second traitement de vieillissement à une température comprise entre 750 et 950°C pendant une période comprise entre 0,5 et 5 heures; et
de refroidissement du moulage en dessous de 600°C à une vitesse de 0,1 à 4°C/mn.
